

## UNITED STATES PATENT OFFICE

2,404,461

METHOD FOR OPERATING BLAST  
FURNACES

Stanley A. Sanford, Cleveland, Ohio

No Drawing. Application October 6, 1942,  
Serial No. 460,979

1 Claim. (Cl. 75—41)

1.

In the production of pig iron by blast furnace operations, four cardinal factors are involved, namely, the blast, the fuel, the charge, and the composition of the resultant slag. As an intermediate and almost equally important factor, there may be mentioned that the chemical composition of the gases coming from the top of the furnace is of importance, as such composition is an indication of the actual performance of the furnace with respect to the volatilization of all the elements which are volatilizable. A consideration of standard text books and prior art could lead the average layman to believe that all ferrous metallurgy, including blast furnace operations, has been reduced to an exact science, that all the important factors involved have been compensated, and that all of these factors in actual performance customarily are dovetailed so completely that the entire operation of a blast furnace is wholly standardized on a basis upon which anyone skilled in the art can duplicate any furnace performance at will. However, this actually has not been the case, standard operations being accompanied by many variations in operating conditions in the same furnace, producing unbalanced chemical and thermal environments, and causing, generally, sub-standard yields which very often fall very substantially below even the rated tonnage of the furnace.

The present invention has for one of its objects the provision of an improved process of blast furnace operation which obviates the irregularities of blast furnace operations which characterize the so-called "standard practice," the present process being distinguished from standard practice by proportioning and maintaining the carbon content of the charge to the oxygen content of the predetermined blast volume in the ratio of more than one pound of carbon for each one pound of oxygen, proportioning and maintaining the iron content of the charge to the carbon content of the charge in the ratio of more than 1.37 pounds but less than 1.82 pounds of iron to each one pound of carbon, proportioning and maintaining the iron content of the charge to the oxygen content of the blast in the ratio of more than 1.37 but less than 1.82 pounds of iron to each one pound of oxygen in the predetermined blast, such proportioning being readily accomplished by dividing the predetermined blast volume by the following empirical division, all

2.

of which are expressed or are inherent in Table II hereinafter set forth in this specification:

- 56.5 for determining the weight of oxygen in the blast per minute;  
5 51.0 for determining the weight of carbon in the charge per minute;  
31.0 for determining the weight of iron in the charge per minute;  
10 75.1 for determining the weight of carbon that will be consumed by the oxygen of the blast per minute;

thereby establishing and maintaining chemical balance upon stoichiometric proportioning, in 15 which not more than 76 per cent of the total weight of carbon in the charge is consumed by the total weight of oxygen in the predetermined blast volume upon the chemical equivalence ratio of 1.33 pounds of oxygen for each one pound of 20 carbon, thus evidencing that since no excess blast oxygen is available, overblowing of the furnace is impossible.

The empirical factors 56.5, 51.0, 31.0 set forth above are based upon the fixed blowing rate of 25 65,000 cubic feet of wind which has been found, in accordance with the present invention, to be the standard requirement of blast for the production of one gross ton of pig iron per minute.

These empirical factors are used as empirical 30 divisions of 65,000 cubic feet to determine the total pounds (per gross ton of pig iron) of the carbon in the coke, iron in the metallic mix of the burden, thus standardizing all critical factors of blast and burden solely upon the blast volume 35 of 65,000 cubic feet per gross ton of iron.

Of the above factors, factor 56.5 is obtained 40 by dividing 65,000 cubic feet of blast per minute by the weight of oxygen in pounds per minute in that blast; the factor 51.0 is obtained by dividing cubic feet of blast per minute by the pounds of carbon in the charge required per minute to unite with the oxygen reaching the tuyères; the factor 31.0 is obtained by dividing 65,000 cubic 45 feet of blast by 2,100 pounds of metallic iron charged per minute; the factor 75.1 is obtained by dividing 65,000 cubic feet of blast by 865 pounds of carbon that are required to combine with 1,150 pounds of oxygen in the 65,000 cubic feet of blast.

50 It is a further object to provide a method of operation which will require a less total weight

of blast than of charge, and a less total weight of oxygen in the blast than of carbon in the charge.

It is a still further object to provide a method of operation whereby the fuel consumption is lowered and furnace production is increased.

It is an additional object to provide a stabilized method of operation which will prevent hanging and slipping of the furnace charge and prevent the creation of "hot tops" and/or "cold bottoms."

**PRESENT IMPROVED METHOD FOR OPERATING BLAST FURNACES**

In accordance with the present invention, it has been discovered that the real timing element in blast furnace operation is the blast, and that maximum temperature of the blast is an imperative adjunct of the blast; that it is equally requisite that the actual percentage of the total carbon that actually arrives at the tuyères for combustion by the oxygen of the blast, be chemically balanced against the actual percentage weight of the oxygen in the blast; and that, very definitely, no blast volume should be blown for the combustion at the tuyères of the remaining percentage of the solid carbon in the charge, because it has been discovered that such remaining percentage weight of carbon undergoes "direct" combustion in the top half of the blast furnace, and, consequently, it never arrives in the combustion zone at the tuyères. Thus, by the present invention, there is eliminated the long standing universal custom of "over-blowing." In fact, it has been found that the entire reduction of iron oxides is accomplished by the process of the present invention, in the top third of the furnace.

In practicing the present invention, it is found that the actual chemistry and the actual mode of reduction tend generally towards 100 per cent thermal efficiency in blast furnace operation only when, insofar as is possible, there is maintained a constant burden ratio and a constant blast volume at maximum temperature, for any given grade of pig iron product; and that any necessary thermal adjustments can be made readily by alteration of the blast temperature, which procedure is in sharp contrast with the long established, universal custom of variations and "over-blowings" which characterize the standard practice, and which continue to unstabilize blast furnace operations.

In accordance with the present invention, the improved results are due to the maintenance of ratios of essential materials in strict chemical equivalence with each other, and because, in the improved process every cardinal factor is established permanently upon a chemical balance of the vital factors O/C/Fe.

It is apparent also that the constant minimum required volume of blast at the maximum temperature would produce the constant minimum products of combustion and, therefore, would convey the constant minimum volume of temperature out of the tuyère zone. Conjointly, the constant minimum fuel ratio would insure the constant minimum products of combustion. Therefore, there is the necessity for the constant minimum required blast volume at maximum temperature and the constant maximum burden ratio, which are the important factors of the present invention.

In accordance with the present invention, it has been determined that the excess blast result-

ing from the variations in the composition of the charge and combustion of the coke in the charge (this excess blast requiring the addition of compensating carbon or, alternatively, reducing the amount of blast being introduced) are undesirable conditions which are to be avoided. This condition causes reduced efficiency, and, in accordance with the present invention there is maintained continuously a chemical balance of the vital components in the charge and in the blast. Such a chemical balance insures maximum production at minimum cost.

It is absolutely necessary that this blast be heated to a temperature as close as possible to 15 1300° F., in order to provide the indispensable back-log of sensible heat that is demanded for continuous operation. Therefore, the prerequisites for obtaining the maximum thermal efficiency of a given furnace are:

20 (1) Determining the maximum rate of carbon combustion per minute, maintained at the tuyères, by blowing a constant volume of blast at maximum temperature.

25 (2) Charging only such total weight of carbon as will insure the arrival at the tuyères of only the requisite total weight of carbon necessary for the maintenance of such established combustion rate;

30 (3) Blowing only, per minute, the total volume of superheated blast, or wind, which contains the necessary oxygen to support the combustion at the tuyères of that proportion of the total weight of carbon. Excess blowing definitely raises the mantle in the furnace and thereby 35 lowers the overall temperature of the hearth, because the increased volume of gases, upon leaving the hearth, carries excessive temperature out of the hearth where it is needed to maintain the indispensable "back-log" for insuring continuous 40 operation, up into the stack where it performs no useful service.

45 The ratio of carbon to oxygen, and the ratio of free oxygen to combined, or reducible, oxygen are vital factors in blast furnace operation. In the foregoing estimates there has been made the very best use of these factors for obtaining the maximum results, wherein the burden ratio would be more than 2.25 and the free oxygen to reducible oxygen ratio should be less than 1.75.

50 In practice it is found that nothing is more fatal to the thermal efficiency of a blast furnace than the long-established and universally used method of "pulling" the wind and decreasing the burden ratio every time the silicon content in the 55 iron threatens to exceed the upper limit of the specification, because this condition of itself is a definite indication of the furnace being over-blown and that the excess volume of hearth gases are carrying the high temperature of the hearth too high in the shaft, thereby inducing the reduction of silica to silicon at a level in the furnace which is considerably above the level at which the oxygen of the blast burns the hearth carbon, that being the level at which the highest 60 temperature should be confined.

65 Blast furnaces that are charged and blasted according to the method herein described obviate the necessity for frequent manipulation, by reason of their ability to adjust themselves automatically to changing conditions within. The following tables show a comparison of the results obtained in practice and in the operation of the present improved process, these furnaces being those to which reference was made previously 70 herein.

Table I

|                                               | Furnace    |                                          |            |                                                                 |
|-----------------------------------------------|------------|------------------------------------------|------------|-----------------------------------------------------------------|
|                                               | "D"        | "D" Operated by present improved process | #5 Western | #5 Western operated in accordance with present improved process |
| Volume of furnace in cu. ft.                  |            |                                          | 39,000     | 39,000                                                          |
| Hearth diameter                               | 21'0"      | 21'0"                                    | 25'0"      | 25'0"                                                           |
| Area of the hearth in sq. ft.                 | 346.4      | 346.4                                    | 490.9      | 490.9                                                           |
| <i>Charge</i>                                 |            |                                          |            |                                                                 |
| Burden ratio                                  | 1.92       | 2.32                                     | 2.50       | 2.85                                                            |
| Gross tons pig iron per day (1440')           | 721        | 1,142                                    | 1,049      | 1,440                                                           |
| Minutes per gross ton                         | 2.00       | 1.28                                     | 1.37       | 1.00                                                            |
| Total weight of charge per minute             | 3,500      | 5,100                                    | 4,690      | 6,375                                                           |
| Total per cent of iron per minute             | 29.50      | 32.32                                    | 32.55      | 33.00                                                           |
| Total pounds of iron per minute               | 925        | 1,670                                    | 1,580      | 2,100                                                           |
| Total per cent of carbon per minute           | 24.30      | 20.00                                    | 22.38      | 20.00                                                           |
| Total pounds of carbon per minute             | 817        | 1,078                                    | 1,060      | 1,275                                                           |
| Pounds of carbon burned per minute            | 772        | 1,010                                    | 994        | 1,185                                                           |
| Same at tuyères burned per minute             | 600        | 728                                      | 730        | 868                                                             |
| Same at tuyères burned per minute             | 73.00      | 66.00                                    | 70.00      | 62.30                                                           |
| Per cent tot. carbon burned tuyères           | 1,634      | 1,360                                    | 1,438      | 1,275                                                           |
| Pounds carbon per gr. ton pig iron            |            |                                          |            |                                                                 |
| <i>Blast</i>                                  |            |                                          |            |                                                                 |
| Total cu. ft. wind per minute                 | 54,470     | 54,470                                   | 65,000     | 65,000                                                          |
| Total cu. ft. wind per minute required        | 44,870     | 54,470                                   | 54,850     | 65,000                                                          |
| Total cu. ft. wind per minute excess          | 9,600      | 0                                        | 10,150     | 0                                                               |
| Total cu. ft. wind per minute excess per cent | 17.50      | 0                                        | 15.50      | 0                                                               |
| Total cu. ft. wind per pound carbon           | 90.8       | 75.2                                     | 90.0       | 75.2                                                            |
| Same required at tuyères                      | 75.2       | 75.2                                     | 75.2       | 75.2                                                            |
| Total pounds oxygen per minute                | 968        | 968                                      | 1,150      | 1,150                                                           |
| Same required tuyères per minute              | 798        | 968                                      | 970        | 1,150                                                           |
| Pounds oxygen excess at tuyères               | 170        | 0                                        | 185        |                                                                 |
| Per cent of excess                            | 17.50      | 0                                        | 15.50      | 0                                                               |
| Total pounds oxygen/gross ton pig iron        | 1,936      | 1,320                                    | 1,576      | 1,150                                                           |
| Ratio Fe/C                                    | 1.11       | 1.55                                     | 1.46       | 1.64                                                            |
| Ratio Fe/C percentage increase                |            | 38.75                                    |            | 12.32                                                           |
| Ratio Fe/O                                    | 0.95       | 1.72                                     | 1.32       | 1.83                                                            |
| Ratio Fe/O percentage increase                |            | 81.05                                    |            | 38.70                                                           |
| Ratio O/C                                     | 1.18       | 0.99                                     | 1.10       | 0.90                                                            |
| Ratio O/C percentage decrease                 |            | 25.75                                    |            | 18.20                                                           |
| Total pounds of blast per minute              | 4,165      | 4,165                                    | 4,975      | 4,975                                                           |
| Total pounds of blast per minute req.         | 3,430      | 4,165                                    | 4,100      | 4,975                                                           |
| Per cent of excess                            | 17.65      | 0                                        | 18.00      | 0                                                               |
| Total wgt. blast per day (1440')              | 5,999,000  | 5,999,000                                | 7,164,000  | 7,164,000                                                       |
| Total wgt. charge per day (1440')             | 5,119,100  | 7,630,000                                | 6,815,000  | 9,180,000                                                       |
| Per cent of increase in tot. chge             |            | 61.50                                    |            | 35.00                                                           |
| Increase of G. T. pig iron/day                |            | 421                                      |            | 391                                                             |
| Per cent of increase                          |            | 58.45                                    |            | 37.25                                                           |
| Fur. vol. wasted by excess bl., cu. ft.       | 13,850,000 | 0                                        | 14,616,000 | 0                                                               |
| Tot. wgt. of excess blast/day, lbs.           | 1,050,320  | 0                                        | 1,118,600  | 0                                                               |
| Per cent of total blast wgt.                  | 17.50      | 0                                        | 27.50      | 0                                                               |

The above demonstrates that the Western furnace, when operated in accordance with the present improved procedure, will have a burden ratio of 2.85 or greater than 2.25, the burden ratio being the ratio of the total weight of the metallic mix of the charge introduced into the furnace to the total weight of coke in the charge (4133 lbs. metallic mix per gross ton of iron + 1450 lbs. of coke per gross ton of iron = 2.85). It will also have a ratio of total weight of charge to total weight of blast greater than 1.00 (6375 lbs. of charge per gross ton + 4975 lbs. blast per gross ton = 1.28); a ratio of total weight of fixed carbon in the charge to free oxygen in the blast greater than 1.00 (1275 lbs. of carbon in charge per gross ton of pig iron + 1150 lbs. of oxygen in the blast per gross ton of pig iron = 1.11); and a ratio of total weight of oxygen in the blast to the total weight of the reducible oxygen in the charge less than 1.75 (1150 lbs. of oxygen in the blast per gross ton of pig iron + 900 lbs. of reducible oxygen in the charge = 1.28).

Generally speaking, the method of the present invention comprises preparing a charge of hematite ore in natural hydrated condition and containing not less than 40 per cent iron, coke, and limestone, introducing the resulting mixture into a blast furnace and blasting the said mixture with super-heated air, while maintaining a burden ratio greater than 2.25 but less than 3.25, a ratio of total weight of charge to blast greater than 1.00 but less than 3.00, a ratio of total weight

of fixed carbon in the charge to the free oxygen in the blast greater than 1.00, but less than 3.00, and a ratio of total weight of oxygen in the blast to reducible oxygen in the charge less than 1.75, but not less than 0.75.

In taking over any operating furnace, the first consideration, in operating in accordance with the improved process, would be the ascertaining of the established production rate and the maximum available blast, or, preferably, the established maximum operating blast. Practically every charging unit has an unused charging capacity of from about 30 per cent to 50 per cent, so that there is sufficient capacity available to meet the requirements for charging according to the improved process. After these determinations are made then Table II would be consulted for ascertaining the correct weights of carbon and of metallic iron for making up the indicated burden. The analysis of the regular operating burden would be determined, and from such analysis, and upon the basis of the established maximum operating blast, there would be determined a burden in conformity with the chemically balanced requirements outlined in Table II, that is, by dividing the cubic feet of blast per minute by the factor 31.00, and also by the factor 51.00, for the purpose of ascertaining, first, the total weight of the iron in the burden, and, second, the total weight of carbon in the burden. Then there would be determined the respective requirements of the number of charging rounds and the total weight of each

round required for the operation in accordance with the improved procedure. The procedure, then, in taking over a given furnace, is as follows:

First, maintain the blast at the established maximum operating blast rate, at not less than 1200° F.;

Second, charge one coke blank, the total weight of which is equivalent to the total weight of the coke in two regular operating rounds plus a total weight of stone which is equivalent to the total weight of stone that is charged in one regular operating round;

In normal furnace operation the furnace is charged in "rounds" each "round" being composed as follows:

|       | Pounds |
|-------|--------|
| Coke  | 13,000 |
| Stone | 7,000  |
| Ore   | 40,000 |
| Total | 60,000 |

Now, in accordance with the second step of changing a conventionally operating furnace to the present improved process as described above, wherein there have been charged into the furnace 26,000 lbs. of coke (one coke blank, the total weight of which is equivalent to the total weight of the coke in two regular operating rounds) plus 7,000 lbs. of stone (total weight of stone that is charged in one regular operating round). This gives the very large "back-log" of heat required for operation of the furnace. No additional coke blanks are necessary.

Third, begin charging in rounds as follows:

Round 1, which is composed as follows:

|                                                                                            | Pounds |
|--------------------------------------------------------------------------------------------|--------|
| Coke: 100% of that charged into the furnace in regular rounds for normal furnace operation | 13,000 |
| Stone: 50% of that charged into the furnace in regular rounds for normal furnace operation | 3,500  |
| Ore: 25% of that charged into the furnace in regular rounds for normal furnace operation   | 10,000 |
| Total                                                                                      | 26,500 |

Round 2, which is composed as follows:

|                                                                                            | Pounds |
|--------------------------------------------------------------------------------------------|--------|
| Coke: 100% of that charged into the furnace in regular rounds for normal furnace operation | 13,000 |
| Stone: 60% of that charged into the furnace in regular rounds for normal furnace operation | 4,200  |
| Ore: 40% of that charged into the furnace in regular rounds for normal furnace operation   | 16,000 |
| Total                                                                                      | 33,200 |

|         | Coke   | Stone  | Ore    | Total  |
|---------|--------|--------|--------|--------|
|         | Pounds | Pounds | Pounds | Pounds |
| Round 3 | 13,000 | 4,900  | 24,000 | 41,900 |
| Round 4 | 13,000 | 5,600  | 32,000 | 50,600 |
| Round 5 | 13,000 | 6,650  | 38,000 | 57,650 |
| Round 6 | 13,000 | 7,000  | 40,000 | 60,000 |

25 This last is a regular round for normal furnace operation, and is reached gradually, as indicated above. The increased burdening of the blast furnace is based upon a constant weight of coke, thence increasing the weight of ore and stone in successive "rounds." Decreased burdening is accomplished by maintaining a constant weight of coke and decreasing the weight of stone and ore.

35 Stated in another way, the percentages referred to in the above tables are percentages of the various quantities of the materials, coke, stone and ore, that are charged into the furnace in regular rounds for normal furnace operation.

40 The charging, blowing, and operating of a blast in accordance with the chemically balanced present process is illustrated in the following table (Table II), the values in the said table being predicated on the use of hematite ore in natural hydrated condition and containing not less than 40 per cent iron:

Table II

|        | Blow per min.      |               | Charge per min. |             | Minutes per gr. ton iron | Gr. tons iron per day | Pounds carbon burned by blast | Percent total carbon |
|--------|--------------------|---------------|-----------------|-------------|--------------------------|-----------------------|-------------------------------|----------------------|
|        | Blast cu. ft. min. | Pounds oxygen | Pounds carbon   | Pounds iron |                          |                       |                               |                      |
| Gr. T. | 100,000            | 1,774         | 1,960           | 3,235       | 0.650                    | 2,215                 | 1,333                         | 70.0                 |
|        | 95,000             | 1,686         | 1,863           | 3,060       | 0.685                    | 2,100                 | 1,267                         | 70.0                 |
|        | 90,000             | 1,593         | 1,765           | 2,900       | 0.725                    | 1,986                 | 1,200                         | 70.0                 |
|        | 85,000             | 1,505         | 1,668           | 2,750       | 0.765                    | 1,882                 | 1,132                         | 70.0                 |
|        | 80,000             | 1,420         | 1,570           | 2,580       | 0.808                    | 1,780                 | 1,068                         | 70.0                 |
|        | 75,000             | 1,330         | 1,472           | 2,420       | 0.900                    | 1,638                 | 1,000                         | 70.0                 |
|        | 72,500             | 1,285         | 1,421           | 2,335       | 0.912                    | 1,592                 | 966                           | 70.0                 |
|        | 70,000             | 1,240         | 1,375           | 2,260       | 0.944                    | 1,525                 | 932                           | 70.0                 |
|        | 67,500             | 1,195         | 1,325           | 2,180       | 0.982                    | 1,483                 | 900                           | 70.0                 |
|        | 65,000             | 1,150         | 1,275           | 2,097       | 1.000                    | 1,440                 | 865                           | 70.0                 |
| N. T.  | 62,500             | 1,105         | 1,225           | 2,015       | 1.042                    | 1,385                 | 830                           | 70.0                 |
|        | 60,000             | 1,062         | 1,175           | 1,932       | 1.083                    | 1,330                 | 800                           | 70.0                 |
|        | 57,500             | 1,024         | 1,135           | 1,866       | 1.108                    | 1,281                 | 769                           | 70.0                 |
|        | 55,000             | 1,018         | 1,125           | 1,855       | 1.132                    | 1,275                 | 766                           | 70.0                 |
|        | 52,500             | 974           | 1,075           | 1,772       | 1.181                    | 1,200                 | 732                           | 70.0                 |
|        | 50,000             | 928           | 1,025           | 1,690       | 1,240                    | 1,165                 | 700                           | 70.0                 |
|        | 47,500             | 885           | 980             | 1,615       | 1,300                    | 1,107                 | 664                           | 70.0                 |
|        | 45,000             | 840           | 930             | 1,532       | 1,372                    | 1,054                 | 631                           | 70.0                 |
|        | 42,500             | 796           | 882             | 1,450       | 1,444                    | 1,000                 | 600                           | 70.0                 |
|        | 40,000             | 752           | 833             | 1,371       | 1,535                    | 950                   | 566                           | 70.0                 |
|        | 37,500             | 708           | 784             | 1,291       | 1,625                    | 900                   | 532                           | 70.0                 |
|        | 35,000             | 664           | 732             | 1,210       | 1,750                    | 843                   | 498                           | 70.0                 |
|        | 32,500             | 620           | 683             | 1,129       | 1,875                    | 775                   | 464                           | 70.0                 |
|        | 30,000             | 570           | 633             | 1,050       | 1,921                    | 720                   | 432                           | 70.0                 |
|        | 27,500             | 539           | 588             | 974         | 2,187                    | 665                   | 400                           | 70.0                 |
|        | 25,000             | 485           | 541             | 888         | 2,384                    | 610                   | 368                           | 70.0                 |
|        | 22,500             | 442           | 490             | 807         | 2,600                    | 555                   | 336                           | 70.0                 |
|        | 20,000             | 398           | 440             | 726         | 2,930                    | 500                   | 300                           | 70.0                 |
|        |                    | 354           | 392             | 645         | 3,250                    | 445                   | 265                           | 70.0                 |
|        | Empirical divisors | 56.5          | 51.0            | 31.0        |                          |                       | 75.0                          | 70.0                 |

NOTE.—Divide C. F. M. blast by empirical divisors for desired quotients.

All intermediate blowing capacities require the respective, proportionate, intermediate weights of metallic iron and carbon, as indicated herein.

Additionally, the following table (Table III) shows the complete chemical balance of the vital factors concerned in the operation of the blast furnaces shown in Table I, showing a comparison between the conditions as they were in standard operation and as they are operating the chemically balanced present improved process for insuring maximum thermal efficiency.

Table III

|                                               | Furnace<br>"D" | Furnace<br>#5<br>Western |
|-----------------------------------------------|----------------|--------------------------|
| Cu. ft. wind per minute.....                  | 54,470         | 65,000                   |
| Pounds oxygen per minute.....                 | 966            | 1,150                    |
| Pounds carbon per minute.....                 | 817            | 1,050                    |
| Pounds carbon per minute should be.....       | 1,078          | 1,275                    |
| Pounds iron per minute.....                   | 925            | 1,580                    |
| Do.....                                       | 1,760          | 2,100                    |
| Gross tons iron per day.....                  | 721            | 1,049                    |
| Do.....                                       | 1,142          | 1,440                    |
| Minutes per gr. ton.....                      | 2.00           | 1.37                     |
| Do.....                                       | 1.26           | 1.00                     |
| Cu. ft. wind per gr. ton.....                 | 108,940        | 89,050                   |
| Do.....                                       | 65,600         | 65,000                   |
| Pounds oxygen per gr. ton.....                | 1,936          | 1,576                    |
| Do.....                                       | 1,150          | 1,150                    |
| Pounds carbon per gr. ton.....                | 1,634          | 1,438                    |
| Do.....                                       | 1,275          | 1,275                    |
| Pounds carbon per gr. ton saving.....         | 359            | 163                      |
| Pounds oxygen per gr. ton saving.....         | 786            | 429                      |
| Cu. ft. wind per gr. ton saving.....          | 43,940         | 24,050                   |
| Cu. ft. wind per gr. ton saving per cent..... | 40.00          | 27.00                    |

portantly, the operation of a blast furnace by blowing it with a less total weight of blast (pounds of wind per net ton of iron) than its total weight of the solid charge (pounds of wind per net ton of all solids, ore, coke, and limestone) per net ton of iron, and that in the solid charge the total weight of fixed carbon is maintained greater than the total weight of oxygen (that is, the pounds of oxygen in the wind) in the blast.

The following additional data is presented as showing further the advantages arising from the operation of blast furnaces in accordance with the present invention. This operating data was obtained on two blast furnaces operating at Donora, Pennsylvania. Blast furnaces No. 1 and No. 2 were identical in all measurements. The same raw materials were used, the same blowing inventions were employed and the same operating personnel was used on both furnaces, utilizing the same technique and producing the same kind of iron under identical conditions, insofar as was possible. The method of the present invention was used on furnace No. 1, but furnace No. 2 was operated according to the conventional method characterized by many blast volume changes, extra coke charged every fourth charge and frequent burden changes. The marked differences in the operation of the two furnaces are shown clearly by the following operating data.

Table IV

|                                                                                                 | No. 1                | No. 2                      |
|-------------------------------------------------------------------------------------------------|----------------------|----------------------------|
| Period covered by the test.....                                                                 | July, 1942, 31 days. | July, 1942, 31 days.       |
| Total net tons pig iron (basic).....                                                            | 24,552               | 19,778.                    |
| Total net tons pig iron per day.....                                                            | 792                  | 638.                       |
| Total net tons pig iron increase/day.....                                                       | 154                  | 0.                         |
| Total net tons pig iron percent/day.....                                                        | 24.10%               | 0.                         |
| Cu. ft. blast per min.....                                                                      | 43,200 (constant)    | 40,500 to 46,500.          |
| Weight of blast per min.....                                                                    | 3,305# (constant)    | 3098# to 3590#.            |
| Minutes per net ton pig iron.....                                                               | 1.83                 | 2.28.                      |
| Cu. ft. blast per net ton pig iron.....                                                         | 79,050               | 92,380 to 106,700.         |
| Weight blast per net ton pig iron.....                                                          | 6,046#               | 7,067# to 8,163# = 7,996#. |
| Weight of blast oxygen per net ton.....                                                         | 1,403#               | 1,640# to 1,894# = 1,820#. |
| Weight of solid carbon per net ton.....                                                         | 1,429#               | Aver. 1,565#.              |
| Weight of solid carbon per net ton percent increase.....                                        | 0                    | 9.50%.                     |
| Weight of solid carbon ton pig iron burned at tuyères.....                                      | 1,053# = 74%         | 1,167# = 74%.              |
| Wgt. oxygen req. for comp. combustion.....                                                      | 1,403#               | 1,550#.                    |
| Excess blast oxygen.....                                                                        | 0#                   | 289#.                      |
| Overblast equal to.....                                                                         | 0 cu. ft.            | 15,000 cu. ft.             |
| Wgt. of solid chge. per net ton pig iron.....                                                   | 6,192#               | 6,370#.                    |
| Wgt. of blast chge. per net ton pig iron.....                                                   | 6,046#               | 7,996#.                    |
| Cu. ft. of blast per net ton pig iron.....                                                      | 79,050               | 104,500.                   |
| Ratio                                                                                           |                      |                            |
| Ratio burden wgt. of metallic mix to coke.....                                                  | 2.28                 | 1.91 2.25 to 3.25          |
| Ratio wgt. of solid chge. to wgt. of blast.....                                                 | 1.02                 | 0.80 1.00 to 3.00          |
| Ratio wgt. of solid carbon to blast oxygen.....                                                 | 1.02                 | 0.86 1.00 to 3.00          |
| Ratio wgt. of blast oxygen to reducible oxygen.....                                             | 1.70                 | 2.28 .75 to 1.75           |
| Ratio pounds of Fe per 1# C.....                                                                | 1.30                 | 1.17.                      |
| Ratio pounds of Fe per 1# C percent increase.....                                               | 11.11%               | 0.                         |
| Ratio CO to CO <sub>2</sub> in top gases.....                                                   | 1.41                 | 2.26.                      |
| Ratio reduction efficiency shown by top gases.....                                              | 1.60                 | 1.00.                      |
| Ratio overall thermal efficiency as shown by the ratio of C to blast oxygen at the tuyères..... | 1.00                 | 0.62.                      |
| Present improved ratios                                                                         |                      |                            |

In accordance with the present invention, there is provided a stabilized operation wherein the reactive elements are all maintained in chemical equivalency throughout the operation, producing substantially greater yields of metal with substantially higher efficiencies of operation and, consequently, reduction in quantities of the reactants, with attendant lowered costs.

It will be seen from the foregoing that the improved process of this invention comprises, im-

70  
Summary of operations on No. 1 and No. 2 blast furnaces at Donora, Pennsylvania, July, 1942.

Both blast furnaces producing basic iron. No. 1 blast furnace operated on present improved method characterized by constancy. No. 2 blast furnace operated on conventional method characterized by frequent changes in blast volume and also in burden ratio due to the charging of extra coke every fourth charge.

## 11

No. 1 produced:

24.10% more pig iron product, using  
9.50% less solid carbon  
25,450 cu. ft. less blast and eliminated  
15,000 cu. ft. of overblast thus demonstrating  
38.00% more overall thermal efficiency and  
60.00% more reduction efficiency as shown by  
the ratio of CO to CO<sub>2</sub> in the top gases and  
also in  
11.10% more metallic iron per pound of solid  
carbon

In the present improved method, all the burden ingredients are weighed in chemical equivalency against the fixed weight of oxygen that is contained in the chosen blast volume in the ratio of 1.33# of oxygen for each 1# of carbon that arrives at the tuyères. Only seventy-five per cent of the total carbon arrives at the tuyères for combustion by the blast oxygen. The remainder of the total carbon charged in the furnace undergoes combustion above the tuyères in the various carbon consuming, direct reactions.

Likewise, 1.25# to 1.81# of metallic iron per each 1# of blast oxygen are charged in the blast furnace burden. These computations are readily made by the use of the factors 31.00 and 51.00 as explained above herein.

Obviously, these ratios are effective only on the basis of constant maintenance of the chosen blast volume and upon a constant burden ratio.

In the conventional method, no similar or equivalent computations are provided, nor indeed can they be because of inconstant blast volume and burden ratio, consequently, chemical equivalency control is never attempted because of the "many variables" that all conventional op-

## 12

erators believe are uncontrollable in blast furnace operations.

It may be pointed out in this connection that in customary operations blast furnace efficiency is based upon the ratio of net tons of pig iron per square foot of hearth area, and the ratio of 2.65 is considered to be representative of good practice.

In accordance with the present invention, regular attainment of ratios of from between 2.90 and 4.90 is experienced by the use of the operating ratios set forth above herein.

This application is a continuation-in-part of co-pending application No. 391,211, filed April 30, 1941.

I claim:

The method of operating a blast furnace for producing pig iron, which comprises preparing a charge including iron ore, coke and limestone, introducing the resulting mixture into a blast furnace, blasting the said mixture to metallic iron with a constant blast of superheated air, while maintaining a burden ratio greater than 2.25, but less than 3.25, a ratio of total weight of charge to blast greater than 1.00, but less than 3.0, a ratio of total weight of fixed carbon in the charge to the free oxygen in the blast greater than 1.00, but less than 3.00, and a ratio of total weight of oxygen in the blast to reducible oxygen in the charge less than 1.75, but not less than 0.75, the said ore being hematite ore in natural hydrated condition and containing not less than 40 per cent iron, and maintaining a constant volume of blast through the tuyères during the entire operation.

STANLEY A. SANFORD.